

## UNITED STATES PATENT OFFICE

2,155,579

DIAZODINITROPHENOL AND METHOD OF  
PREPARATION OF THE SAME

Leon W. Babcock, Kenvil, N. J., assignor to Hercules Powder Company, Wilmington, Del., a corporation of Delaware

No Drawing. Application December 21, 1937,  
Serial No. 181,028

5 Claims. (Cl. 260—141)

This invention relates to a method for the production of diazodinitrophenol, and more particularly to a method whereby diazodinitrophenol may be produced directly in a free-flowing form, adapted for machine loading into blasting caps.

5 Diazodinitrophenol has long been known, as have various methods for its production, e. g. United States Letters Patent to Dehn, Nos. 1,404,087; 1,428,011; 1,460,708. Diazodinitrophenol constitutes a very valuable explosive for use in blasting caps, but, as produced in accordance with the above processes, it is not free-flowing, but composed of needle-like crystals, and hence not adapted to machine loading of blasting caps.

10 Methods of preparation of free-flowing diazodinitrophenol are known, e. g. in accordance with United States Letters Patent Re. 19,645 to Hancock and Pritchett, disclosing a slow rate of addition of acid to the diazotization mixture, and Patent No. 2,103,926 issued December 28, 1937 to Harvey B. Alexander disclosing diazotization in the presence of certain compounds which prevent the formation of needle-like crystals.

15 In accordance with this invention a novel, simple and economical method is provided for the production of diazodinitrophenol, in which diazodinitrophenol may be prepared directly in free-flowing form, without the use of any added materials and without the excessive supervision required by the gradual addition of acid in the Hancock and Pritchett process.

20 In practicing the process in accordance with this invention, the acid is added to the diazotization mixture by means of an atomizer or spraying device, operated by the use of compressed air or other gas inert to the ingredients of the diazotization mixture, such as carbon dioxide, nitrogen, or the like.

25 While the theory of the operation of my new process has not been clarified, I am of the opinion that the advantage of my improved process lies in the elimination of local regions of high acid concentration in the diazotizing bath, practically impossible to overcome with processes used heretofore and involving gradual flow of acid to the diazotization bath. Since rate of diazotization depends upon acid concentration, reaction progresses uniformly throughout the entire mixture

30 in my improved process, building up all crystal agglomerates uniformly at the same rate and producing uniform grain size.

35 Moreover, the elimination of local regions of high acidity prevents the formation of very fine particles of diazodinitrophenol, which form dust

on drying, which fine particles are caused by very rapid diazotization reaction. Dust in dry diazodinitrophenol is a very serious disadvantage, not only in that it hinders free-flowing in machine loading, but constitutes a serious hazard when settling on various apparatus used in the manufacture of blasting caps.

40 Also, the process in accordance with my invention premits the production of diazodinitrophenol of uniform and controlled density, a highly important factor in the manufacture of blasting caps. Diazodinitrophenol manufactured in accordance with processes heretofore known has suffered from unexpected and uncontrollable variations in density. Since blasting caps are necessarily loaded by machine and by measured volume of explosive charge, it is evident that a low density diazodinitrophenol will produce a blasting cap having therein a less weight of charge, and vice versa. Heretofore, it has been necessary to blend various lots of diazodinitrophenol, in accordance with their density, in order to produce a material of uniform density suitable for loading into blasting caps. The use of my improved process, producing a product of uniform density, renders such blending unnecessary except in unusual cases.

45 The injector or atomizer used in my process need not be of any particular shape or form, but need only be adapted to atomize the acid used into fine droplets and force the same under the surface of the diazotizing mixture. It should be of acid-resisting material, e. g. glass, porcelain, stoneware, or the like, because it must handle dilute mineral acids. I prefer to use glass as the material of construction, for the reason that porcelain or stoneware are liable to chip or wear and introduce grit into the material formed. The atomizer is preferably placed a short distance below the surface of the diazotizing mixture.

50 In the practical adaptation of my invention, any suitable salt of picramic acid may be used, e. g. sodium picramate, ammonium picramate, magnesium picramate. Likewise, various nitrites, such as sodium nitrite, potassium nitrite, barium nitrite. The acid used may be any suitable acid adapted to effect diazotization of the picramate and nitrite, such as hydrochloric, sulfuric, phosphoric, acetic, etc.

55 In carrying out the method in accordance with my invention, the picramate and nitrite will be in solution or in suspension, or partly in solution and partly in suspension, in water. For example, a suspension of sodium picramate of concentration as high as 9.7% has been success-

5

10

15

20

25

30

35

40

45

50

55

fully diazotized by the method in accordance with my invention, but I do not limit my invention to this percentage. The solution or suspension of picramate will, desirably, be substantially neutral, and the concentration of the picramate therein may vary widely. The temperature during the diazotization will, desirably, be maintained by any suitable means within the range of about 10° C. to about 16° C. The diazotizing mixture will be suitably stirred or agitated, e. g. by a rotating stirrer or by a current of air or gas inert to the mixture being diazotized.

As illustrative of the practical application of the method in accordance with this invention, about 61.2 pounds, dry weight, of water-wet sodium picramate, screened to remove foreign material, is charged into a diazotizing tub, preferably of wood, fitted with a stirrer, and about 90 gallons of water added. About 19 pounds of sodium nitrite, dissolved in about 10 gallons of water, are then run into the diazotizing tub, and the stirrer started. The temperature of the mixture is then brought to the desired point, e. g. about 15° C. Then about 40 liters of 20% hydrochloric acid are sprayed or atomized into the mixture, under the surface of said mixture, by the use of the atomizer heretofore described, preferably at such a rate as to require about 275 minutes to add the entire amount of acid. The rate of addition of the acid may be varied considerably, depending upon the pressure of the compressed gas used in the atomization. About 5 minutes after completion of addition of the acid, the mixture is tested with potassium iodide-starch test paper, and, if such test shows a strong, positive indication of excess of nitrous acid, diazotization of the sodium picramate is complete.

Stirring is then stopped and the mixture placed on a suction filter, the mother liquor drawn off, and the diazodinitrophenol washed with water.

The method in accordance with this invention is not dependent upon the use of any particular form or size of apparatus, means for cooling, or the like.

What I claim and desire to protect by Letters 5 Patent is:

1. The method for producing diazodinitrophenol in a free-flowing form which includes diazotizing a picramate in the presence of a nitrite and water by adding thereto acid in 10 atomized form beneath the surface of said picramate, nitrite and water.

2. The method for producing diazodinitrophenol in a free-flowing form which includes diazotizing a substantially neutral mixture of a 15 salt of picramic acid, a nitrite, and water by addition thereto of an acid in atomized form beneath the surface of said picramate, nitrite and water.

3. The method for producing diazodinitrophenol in a free-flowing form which includes diazotizing a picramate by addition thereto of an acid in atomized form beneath the surface of the reaction mixture, in the presence of a nitrite and water, while maintaining the temperature of the reactants within the range of 25 about 10° C. to about 16° C.

4. The method for producing diazodinitrophenol in a free-flowing form which includes diazotizing sodium picramate by addition there- 30 to of hydrochloric acid in atomized form beneath the surface of the reaction mixture, in the presence of sodium nitrite and water.

5. The method for producing diazodinitrophenol in a free-flowing form which includes 35 diazotizing sodium picramate by addition thereto of hydrochloric acid in atomized form beneath the surface of the reaction mixture, in the presence of sodium nitrite and water, while maintaining the temperature of the reactants 40 within the range of about 10° C. to about 16° C.

LEON W. BABCOCK.